# EUROPEAN PATENT SPECIFICATION

(11) **EP 0 050 969 B1**
(45) Date of publication and mention of the grant of the patent: **04.07.1984**
(21) Application number: 81305004.4
(22) Date of filing: 23.10.1981
(51) Int. Cl.: C22C 33/02

(54) **Alloy steel powder**
Legiertes Stahlpulver
Poudre d'acier allié

(30) Priority: 24.10.1980 US 200527
(43) Date of publication of application: 05.05.1982
(73) Proprietor: AMSTED Industries Incorporated, Chicago, IL. 60601 (US)
(72) Inventor: Lynn, Jean C., Chicago Illinois 60601 (US)
(74) Representative: Skailes, Humphrey John

## Description

The present invention provides a corrosion resistant iron base alloy powder and a method of producing final products using the same. More specifically, the alloy powder is a modification of a type 300 series stainless steel, with increased percentages of silicon and phosphorus. The alloy powder is useful for producing fully dense metal products by powder metallurgy techniques.

Type 300 series stainless steels are common stainless steels used in numerous industrial applications. In attempting to make fully dense products from the atomized powder of the alloys of this type of stainless steel using powder metallurgy techniques, it is known that powder alloys of the typical compositions of the alloy series, i.e. type 304 and type 316, are difficult to sinter to full density.

It is believed that the difficulty in sintering is due to the narrow difference between the solidus and liquidus temperatures of these alloys. This difference is approximately 10°F (5°C). Accordingly, the width of the liquid phase sintering range of such an alloy would be so narrow that it would be economically impractical to control the sintering temperature accurately enough in a commercial production operation.

Accordingly, it is necessary to increase the difference between the liquidus and solidus temperatures in order that liquid phase sintering can be commercially performed.

The present invention provides a high alloy steel powder useful in forming fully dense, corrosion resistant products by powder metallurgy techniques. A method of producing final products from the steel powder is also provided.

In the method of producing the alloy powder of the present invention, the typical composition of the type 300 series stainless steel is changed to provide additional silicon and phosphorus. Thus the invention provides an alloy steel powder containing, by weight:

the balance being iron, apart from unavoidable impurities.

The difference between the solidus and liquidus temperatures is increased to greater than 25°F (14°C) by the addition of the silicon and phosphorus, and sintering can be commercially performed within the temperature range. The additional silicon is usually added in a pre-alloy operation prior to atomization of the molten alloy to form a powder. The phosphorus can be added in the pre-alloy operation, but can also be added in the pre-alloy operation, but can also be added in an ad-mix operation. In such an ad-mix operation, the phosphorus is added in powder form to the alloy powder, usually in the form of ferro-phosphorus powder.

The nickel content of the alloys is preferably about 12%. The silicon content may for example be 2-3% and is preferably about 3%. The phosphorus content is preferably 0.08-0.1 %.

The maximum carbon content of the alloys is typically about 0.1%, and if desired carbon, manganese and molybdenum can be absent from the compositions.

The invention is illustrated in the following examples:

### Example 1

One iron base alloy that was water atomized and screen at -88 mesh to provide a powdered metal had the following initial analysis by weight:

The powdered metal was blended with about 1% by weight Acrawax (Trademark) for die lubrication purposes. Any similar lubricant may also be used. The sample was compacted in a die at 50 TSI (7047 Kg/cm²), the lubricant was removed in a burn off process and then the compacted sample was vacuum sintered at 2420°F (1327°C) for 90 minutes. A final product of over 97% theoretical density, ultimate tensile strength of 100,000 Ib/in² (7047 Kg/cm²), yield strength of 49,000 Ib/in² (3452 Kg/cm²), elongation of 10% and unnotched impact strength of 32 ft-Ib (43 joules) was produced. In addition, the corrosion rate of the final product was 0.1 inch per year (0.25 cm/year). The corrosion test was performed according to practice B of ASTM A 262. The product was also found to be rust free in a 5% salt fog environment according to ASTM B 117-63.

If desired, the final products can be water quenched to improve corrosion resistance, ductility, toughness and other properties. In the above example, the final product when water quenched from a solution treatment temperature of 2100°F (1150°C) has an elongation of 40% and an unnotched impact strength of greater than 120 ft-Ib (163 joules). The corrosion rate of the final product was 0.04 in/yr (1 mm/yr) in boiling sulfuric acid according to practice B of ASTM A 262.

Other samples of similar composition were successfully sintered at temperatures between 2380-2460OF (1305-1350⁰C).

### Example 2

Another iron base alloy that was water atomized and screened at -88 mesh to provide a powdered metal had the following initial analysis by weight:

The powdered metal was compacted and sintered in a manner similar to Example 1. The final product had properties similar to the final product in Example 1, except that elongation improved to 26%. The corrosion rate was 0.047 in/yr (1.2 mm/yr).

### Example 3

Another iron base alloy that was water atomized and screened at -88 mesh to provide a powdered metal had the following initial analysis by weight:

The powdered metal was blended with about 1% by weight Acrawax (Trademark) for die lubrication purposes. Any similar lubricant may also be used. The sample was compacted in a die at 50 TSI (7047 Kg/cm²), the lubricant was removed in a burn off process and then the compacted sample was vacuum sintered at 2430°F (1332°C) for 90 minutes. A final product of 99% theoretical density, ultimate tensile strength of 93,000 Ib/in² (6553 Kg/cm²), yield strength of 37,000 Ib/in² (2607 Kg/cm²), elongation of 45%, unnotched impact strength of greater than 120 ft-Ib (161 joules) and notched impact strength of 17 ft-Ib (23 joules) was produced.

In this example, when the final product was gas fan cooled from a solution treatment temperature of 2100°F (1150°C) it has an elongation of 57% and a notched impact strength of 38 ft-in (51 joules). The corrosion rate was 0.16 in/yr (4 mm/yr).

### Example 4

Another iron base alloy that was water atomized and screened at -88 mesh to provide a powdered metal had the following initial analysis by weight:

The powdered metal was compacted and sintered in a manner similar to that set forth in Example 1. The final product had properties similar to the final product in Example 1, except that the corrosion rate was 0.05 in/yr (1.27 mm/yr).

### Example 5

Another iron base alloy that was water atomized and screened at -88 mesh to provide a powdered metal had the following initial analysis by weight:

The powdered metal was compacted and sintered in a manner similar to that set forth in Example 1. The final product has properties similar to the final product in Example 1, except that the corrosion rate was 0.037 in/yr (0.94 mm/yr).

### Example 6

Another iron base alloy that was atomized and screened at -88 mesh to provide a powdered metal had the following initial analysis by weight:

The powdered metal was compacted and sintered in a manner similar to that set forth in Example 1. The final product had properties similar to the final product in Example 1, except that the corrosion rate was 0.049 in/yr (1.25 mm/yr).

### Example 7

Another iron base alloy that was water atomized and screened at -88 mesh to provide a powdered metal had the following initial analysis by weight:

The powdered metal was compacted and sintered in a manner similar to that set forth in Example 1. The final product had properties similar to the final product in Example 1.

### Example 8

Another iron base alloy that was water atomized and screened at -88 mesh to provide a powdered metal had the following initial analysis by weight:

The powdered metal was compacted and sintered in a manner similar to that set forth in Example 1. The final product had properties similar to the final product in Example 1, except that the corrosion rate was 0.10 in/yr (2.5 mm/yr).

## Claims

1. An iron base alloy powder containing, by weight:
the balance being iron, apart from unavoidable impurities.

2. An alloy powder as claimed in claim 1 which contains about 12% nickel.

3. An alloy powder as claimed in claim 1 or claim 2 which contains 2-3% silicon.

4. An alloy powder as claimed in any one of the preceding claims which contains about 3% silicon.

5. An alloy powder as claimed in any one of the preceding claims which contains 0.08―0.1% phosphorus.

6. An alloy powder as claimed in any one of the preceding claims which contains up to about 0.1% carbon.

7. An alloy powder as claimed in claim 1 having by weight, any one of the compositions set out below:
the balance in each case being iron, apart from unavoidable impurities.

8. Products produced by compacting and sintering a powder as claimed in any one of the preceding claims.

## Patentansprüche

1. Eisenbasislegierung in Pulverform enthaltend bezogen auf auf das Gewicht:
wobei der Rest, abgesehen von unvermeidbaren Verunreinigungen, Eisen ist.

2. Legierung in Pulverform gemäß Anspruch 1, dadurch gekennzeichnet, daß sie etwa 12 % Nickel enthält.

3. Legierung in Pulverform gemäß Anspruch 1 oder 2, dadurch gekennzeichnet, daß sie 2 bis 3 % Silicium enthält.

4. Legierung in Pulverform, wie in einem der vorhergehenden Ansprüche beansprucht, dadurch gekennzeichnet, daß sie etwa 3 % Silicium enthält.

5. Legierung in Pulverform, wie in einem der vorhergehenden Ansprüche beansprucht, dadurch gekennzeichnet, daß sie 0,08 bis 0,1 % Phosphor enthält.

6. Legierung in Pulverform, wie in einem der vorhergehenden Ansprüche beansprucht, dadurch gekennzeichnet, daß sie bis zu etwa 0,1 % Kohlenstoff enthält.

7. Legierung in Pulverform, wie in Anspruch 1 beansprucht, mit einer der folgenden Zusammensetzungen bezogen auf das Gewicht:
wobei der Ausgleichsrest in jedem Fall, abgesehen von unvermeidlichen Verunreinigungen, Eisen ist.

8. Produkte, hergestellt durch Kompaktieren und Sintern eines Pulvers, wie in einem der vorhergehenden Anssprüche beansprucht.

## Revendications

1. Alliage à base de fer, en poudre, contenant (pourcentages en poids):
le solde, à part d'inévitables impuretés, étant du fer.

2. Alliage en poudre suivant la revendication 1, contenant environ 12 % de nickel.

3. Alliage en poudre suivant la revendication 1 ou la revendication 2, contenant de 2 à 3 % de silicium.

4. Alliage en poudre suivant l'une quelconque des revendications précédentes, contenant environ 3 % de silicium.

5. Alliage en poudre suivant l'une quelconque des revendications précédentes, contenant de 0,08 à 0,1 % de phosphore.

6. Alliage en poudre suivant l'une quelconque des revendications précédentes, contenant jusqu'à environ 0,1 % de carbone.

7. Alliage en poudre suivant la revendication 1, possédant l'une quelconque des compositions ci-après (% en poids):
le solde, à part d'inévitables impuretés, étant dans chaque cas du fer.

8. Produits fabriqués par compactage et frittage d'une poudre suivant l'une quelconque des revendications précédentes.
